

Oct. 9, 1928.

1,687,042

P. C. SEEL

ANTISTATIC PHOTOGRAPHIC FILM AND FILM BASE THEREFOR

Filed Aug. 12, 1927



Paul C. Seel,  
INVENTOR,  
BY R. L. Stinchfield  
ATTORNEY

## UNITED STATES PATENT OFFICE.

PAUL C. SEEL, OF ROCHESTER, NEW YORK, ASSIGNOR TO EASTMAN KODAK COMPANY, OF ROCHESTER, NEW YORK, A CORPORATION OF NEW YORK.

## ANTISTATIC PHOTOGRAPHIC FILM AND FILM BASE THEREFOR.

Application filed August 12, 1927. Serial No. 212,569.

This invention relates to antistatic photographic film and to the base or support thereof. One object of the invention is to provide such a film which will have the usual qualities required to meet commercial conditions and will have, in addition, the ability to prevent or greatly lessen defects due to electrical discharges which are customarily referred to as "static" markings. Other objects will hereinafter appear.

In the accompanying drawing the single figure is a diagrammatic section, upon an enlarged scale, of a photographic antistatic film embodying my invention.

I have found that a photographic film in which the light-sensitive photographic layer, such as a gelatino-silver-halide emulsion, is carried by an electrifiable base or support, can be rendered substantially antistatic by providing it with a layer or backing containing an abietic acid ester. This backing is on the face of the support opposite to the one carrying the emulsion. Only a very thin layer, relative to the thickness of the support, is required to bring about the antistatic result. It is, therefore, comparatively inexpensive to carry out my invention.

In the preferred form of my invention, which will be described in detail by way of illustration, I dissolve 3 parts by weight of the abietic acid ester in 97 parts by weight of acetone. The surface of the support to be coated is then brought very rapidly into and out of contact with this solution, so as to evenly and thoroughly coat it with a very thin layer. The acetone rapidly evaporates, leaving a sufficiently hard backing, and yet the acetone insures a strong bond between the abietic acid ester coating and the pyroxylin or other electrifiable film support. Of course, in place of acetone any other volatile solvent, common to the electrifiable support and the abietic acid ester, can be employed.

Referring to the accompanying drawing, 1 is a light-sensitive photographic layer, such as a gelatino-silver-halide emulsion,—say a negative motion picture emulsion. 2 is the electrifiable film support, such as a transparent, flexible, strong, waterproof, pyroxylin layer, like that customarily employed in motion picture film. 3 is the antistatic layer or backing containing the abietic acid ester. It remains unaffected by the photographic baths.

While I may employ various esters of abietic acid with different alcohols, I prefer to use the glyceryl ester of this acid, which is available commercially in a form resembling copal. In the thin layers which I use it is substantially colorless, flexible and transparent. Since static manifestations are most apt to occur upon developing motion picture negative film that has been exposed under particularly dry atmospheric conditions, my invention is at the present time of most utility in rendering such film antistatic.

Having thus described my invention, what I claim as new and desire to secure by Letters Patent is:

1. A flexible, photographic film comprising an electrifiable support carrying on one face a light-sensitive photographic coating and on the other face an antistatic layer containing an abietic acid ester.

2. A photographic film comprising a nitrocellulose support carrying on one face a gelatino-silver-halide emulsion and on the other face an antistatic layer containing an abietic acid ester of glycerol.

3. A flexible, transparent base or support adapted to receive light-sensitive photographic coatings, which comprises a main nitrocellulose layer and a relatively thin coating of an abietic acid ester of glycerol.

Signed at Rochester, New York, this 4th day of August, 1927.

PAUL C. SEEL.